# EUROPEAN PATENT SPECIFICATION

(11) **EP 1 264 706 B1**
(45) Date of publication and mention of the grant of the patent: **19.07.2006**
(21) Application number: 02011821.2
(22) Date of filing: 28.05.2002
(51) Int. Cl.: B41M 5/035

(54) **Transfer printing process**
Übertragungsdruckverfahren
Procédé d'impression par transfert

(30) Priority: 07.06.2001 IT MI20011198
(43) Date of publication of application: 11.12.2002
(62) Divisional of application: 06008732.7
(73) Proprietor: Menphis S.p.A., 22070 Casnate con Bernate (Como) (IT)
(72) Inventor: Menin, Gilberto, 22070 Montano Lucino, Como (IT)
(74) Representative: Sama, Daniele

(56) References cited:
- EP-A- 0 921 014
- EP-A- 0 953 457
- EP-A- 1 092 550

## Description

The present invnetion relates to a transfer printing process employing a particular composite which can be used in the bag tecnique, as described hereafter, to obtain a drawing reproduction wuth a very good picture definition, very good chromatic yield and substantially defect free, such as bubbles, dots, uncompactness, etc.

More specifically in the transfer printing of the invention the colour transfer is made by sublimation and a particular composite film is used comprising a mated polymer film having a metallized surface on which a drawing, preferably coloured, is printed.

More in particular said process is applied to flat surfaces and tridimensional articles and is carried out under reduced pressure, optionally by treating the composite, before the printing, with conventional techniques so that the composite results electrostatically charged.

Still more in particular the process of the present invention uses a composite comprising a basic polymer film having one or both the surfaces mated, i.e., opaque and rough, wherein a mated surface is metallized and on the metal layer a drawing, preferably coloured, is printed by sublimable inks at the temperatures of the transfer printing process.

The transfer printing is a consolidated and diffused printing technique in the industries of this field.

Compared with the conventional printing, the transfer printing shows the following advantages:
- more faithful reproduction also of high complexity drawings (four-colour process);
- lower printing costs, since less sophisticated colour transfer plants are required;
- reduced environmental impact, the total amount of colours dispersed in the environment being very low;
- as regards the printing on textiles, elimination of the vaporization, washing and finishing phases used in the conventional printing, and therefore elimination also of the respective processing recycling.

By using the transfer printing technique the drawing is first printed, for example by rotogravure printing, on a suitable support; subsequently the drawing transfer is carried out on the manufactured article, for example by calendering for textiles or by heating in an oven for aluminum profiles or articles of various shapes, at temperatures in the range 170°C -240°C. At said temperatures the transfer step is complited in some minutes.

In European patent application EP 921,014 in the name of the Applicant, a composite for transfer printing is described, formed by a basis polymer layer on which a thin aluminum layer is deposited. On the aluminum surface the drawing is printed by sublimable colours.

The composite can be used to print flat surfaces or tridimensional articles such as aluminum profiles, doors and windows or others. In the patent application it is described that in the tridimensional article printing the so called "membrane" technique can be used, consistsing in coating the article wrapped in the composite in an external membrane. Inside the pocket formed by the membrane, hermetically sealed, vacuum is made. With this printing technique of tridimensional articles, using the above described composite, printed manufactured articles are obtained having a very good chromatic yield and definition of the transferred drawing.

Another technique to print tridimensional articles with drawings having sublimable colours is the so called "bag" technique. Said technique is industrially cheaper than the "membrane" technique, since the printing preparation steps are simpler and the whole cycle is carried out in shorter times. The external pocket, which constitutes the bag, is formed in this case by the same composite film. During the printing step the vacuum is kept by connecting the pocket to a vacuum pump.

The Applicant has found that the transfer printing by the bag technique on tridimensional articles and non, carried out by the composite of the above European patent application, has a lower quality in comparison with the printing obtained in the same conditions by the membrane technique. See the Examples.

The need was therefore felt to have available a transfer printing process by colour sublimation on tridimensional articles and flat surfaces, carried out by means of the bag technology as above defined, such to allow to obtain a manufactured article having the following property combination:
- defect free (bubbles, blurrings in the printed drawing, etc.),
- very good imagine definition and chromatic yield comparable with that obtainable by the membrane transfer printing technique by using the composite of the above European patent application,
- easy transfer with high definition of complex drawings, such for example the drawing of the pinewood grain.

The Applicant has surprisingly and unexpectedly found a process wherein the bag transfer printing technology is used which solves said technical problem.

An object of the present invention is a transfer printing process by colour sublimation by means of the bag technology, comprising the following steps:
a) coating of the article surface to be printed with a composite comprising:
   - a polymer film or sheet, which forms the composite basis and is capable to resist without decomposing and without being deformed at the temperatures used in the colour transfer phase by sublimation, said polymer film or sheet having a thickness ranging from 6 to 100 µm and having one or both the surfaces mated, therefore rough and opaque,
   characterized by a gloss < 60%, determined by the DIN 67530 method with measurement angle of 85°;
   - an aluminum layer, having a thickness fromt 0,5 to 40 nm preferably from 1 to 20 nm preferably having an optical density in the range 0.05-3.0, preferably 0.1-0.5, measured by TD 932 - Macbeth densitometer, the aluminum layer being deposited on a mated surface of the polymer compound film;
   - a drawing, with the respective colours, printed on the aluminum layer and put into contact with the surface of the article to be printed;
b) longitudinal closing of the case formed by the composite and vacuum application or pressure reduction between the composite film and the article to be printed, using a residual pressure from 0.05 bar (5X10³ Pa) to 0.2 bar (2X10⁵ Pa), preferably 0.1 bar (10⁴ Pa);
c) heating at temperatures from 170°C to 240°C, preferably from 190°C to 210°C, keeping the residual pressure within the previous limits, for a time from 1 minute to 5 minutes;
d) cooling and recovery of the printed article.

The longitudinal closing of the case formed by the composite can be carried out for example by adhesive tape, or by ultrasound welding, using known techniques.

The vacuum is applied to the two ends of the case formed by the composite by a pump.

Optionally, the composite can be treated by conventional techniques so that it results electrostatically charged when used in the process according to the present invention. In this way the adhesion of the composite to the article is easier and therefore the bag formation and the vacuum application is simpler.

To carry out the printing process, for example an oven suitable to this purpose or any other equivalent equipment can be used.

The thickness of the polymer compound film is preferably from 10 to 25 micron and the optical density of the aluminum film, determined as above, is preferably from 0.1 to 0.5.

Preferably the gloss of the rough surface of the polymer film forming the basis composite film, is > 10%, measured by the above method, but with contact angle of 60°, still more preferably it ranges from 15%, measured with angle of 60° to 55%, measured with angle of 85°, extremes included.

The polymer forming the film or sheet is selected from polyesters, fluorinated resins, polyamides, polyimides, polyethers and polyurethane resins.

Preferably a polymer film of polyester, in particularl polyethylene terephthalate, polybutylene terephthalate, glycol terephthalate is used.

Also polymer films stretched in one or both the directions, longitudinal and/or transversal, can be used.

The results obtained with the composite of the present invention are surprising since tests carried out by the Applicant have shown that by using only the basis polymer film, with the mated surface, the transferred imagine definition and the chromatic yield are not satisfactory.

Furthermore the use of the composite of the present invention allows a significant time reduction of the transfer printing process, contemporaneously using lower temperatures and lower times with respect to non metallized mated films.

The preparation process of the composite film used in the process of the present invention takes place in two steps.

In the first step the mated polymer film is prepared.

This step can be carried out according to known methods, for example by extrusion of the polymer containing inorganic fillers, or by chemically or mechanically treating, for example by embossing or by applying a resin layer on one or both the film surfaces, or by the "crown" treatment using well known methods to the skilled man in this field.

Mated polymer films are easily available both by the plastic compound manufacturers and on the market.

The mated films are indeed largely used for the flexible packages.

The metallization of the mated surface of the polymer film is carried out by deposition of an aluminum layer under high vacuum conditions, using the usual techniques well known to the skilled man in this field.

The film is printed with the drawing to be transferred on the side coated with aluminum, by using offset, flexo, rotogravure, serigraphy printing machines, preferably a rotogravure printing machine is used.

The used inks are those usually available on the market and that can be emulsifiable or disperseable in water or in solvent and must preferably be of the type having high resistance to light.

With the composite film according to the present invention both flat surfaces and tridimensional articles, even with irregular surfaces, can be printed.

As said, the colour transfer on the final support according to the process of the present invention is carried out by the colour sublimation technique at temperatures preferably from 190°C to 210°C.

The contact time is generally from 1 minute to 5 minutes, and varies depending on the article mass and on the thermal exchange process conditions during the transfer step.

The transferred colour amount is of the order of 90% or higher.

As said, in the printing of tridimensional articles or flat surfaces, the image definition results comparable with that obtained by using the metallized composite of the prior art in the membrane transfer printing technique under vacuum.

Generally the invention films can be used for the transfer printing by applying them to any article to be printed formed by a compound resistant to the temperatures used in the printing process by sublimation and having surfaces capable to absorb the sublimable colours which are transferred from the metallized composite surface.

According to a preferred embodiment of the present invention process the surfaces of the support to be printed are previously coated, for example by electrostatic painting, with a layer of polymer compound, for example polyester or polyurethane thermosetting powders, formulated so to favour the sublimable ink maximum penenetration.

The composite films of the present invention can be used for the transfer printing technique for the application to supports formed by different materials, for example metals (aluminum, iron, zinc, steel, cast iron), or glass, ceramic, or polymer compound manufactured articles.

The materials can have the form of both flat surfaces and tridimensional articles.

It has been found by the Applicant that by using the invention composite at the temperatures used in the transfer printing process, the drawing does not result deformed when it is printed on the manufactured article. This represents a remarkable advantage since the articles to be discarded for said printing defect are practically absent.

The process according to the present invention is much more unexpected if one considers that the use of the only mated film in the transfer printing by colour sublimation does not allow to obtain a very good imagine definition. See the comparative Examples.

Another object of the present invention is the composite used in the printing process which has been described above.

The following Examples have the purpose to illustrate the invention and are not to be intended as limitative of the scope of the same.

### EXAMPLE 1 (comparative)

Use of the composite according to the European patent application EP 921,014 in the transfer printing by means of the bag technology

An unmated polyethyelenterephthalate film (gloss = 100%) having a thickness of 23 µm metallized on one side with aluminum having a thickness of 12,5 nm, corresponding to an optical density determined by densitometry of 2.1 (metallized film A) is printed with a colour drawing reproducing the pinewood grain.

The receiving support is an aluminum profile for door and windows, having sizes of about 7 meters x 10 cm x 5 cm, pretreated by electrostatic painting with polyester thermosetting powdered paint having a thickness of 75 micron.

The composite film is wrapped around the profile, so that folds do not form, and hermetically sealed on the longest side. By a pump a vacuum of 0.1 bar (10⁴ Pa) is made, taking care that folds or bubbles between the composite and the article do not form. The transfer printing is effected by transferring the wrapping wrapped on the aluminum profile in an oven at 205°C for 4 minutes, keeping the vacuum at the above indicated value by means of the pump.

At the end it is cooled, the atmospheric pressure is restored and the composite film is taken away from the article.

The drawing printed on the aluminum bar (Fig. 1) shows printing defects attributable to air bubbles or non evacuated vapors, which have prevented the film from contacting the paint layer on the profile. Besides, some particulars of the printed grains result blurred. Therefore the reproduction of the printed drawing is not good. It is observed that on the used composite only traces of the sublimable inks remain. Therefore the colour transfer on the aluminum bar has been substantially quantitative.

### EXAMPLE 2

Transfer printing by the bag technology using a composite wherein the basis polymer film surface is mated and has a gloss of 45%

Example 1 is repeated but by using a composite film in which one of the basis film surfaces is mated and then it has been metallized with aluminum.

The mated surface has a gloss of 45% determined by the DIN 67530 method, by using a measurement angle of 85°.

The drawing printed on the aluminum bar (Fig. 2) does not show defects (no air bubbles or blurrings) and it is of a very good quality. It is observed that on the used composite only traces of the sublimable inks remain. Therefore the colour transfer on the aluminum bar has been substantially quantitative.

If Figures 1 and 2 are compared, one clearly sees that the drawing reproduction in the case of Figure 2 is evidently higher than that obtained in Figure 1.

### EXAMPLE 3 (comparative)

Printing with the bag technology using only the mated basis film.

Example 2 is repeated but by using only the mated basis polymer film (not metallized with the aluminum layer) on which the same colour drawing is printed.

The drawing printed on the aluminum profile (Figure 3) in this case shows a lower definition than that obtained in Example 2. At the visual observation it is noticed that the lines reproducing the grains are discontinuous, mostly formed by a sequence of points: the drawing shows the printing defect known as "uncompactness" and it is not of an acceptable quality.

It is noticed that on the polymer film recovered at the end of the process an evident amount of inks remains, such that the original drawing is easily recognizable. Therefore by using only the mated polymer film in the transfer printing process with the above mentioned technique, the colours are only partially transferred to the support.

### EXAMPLE 4

Transfer printing by the bag technology by using a composite in which the basis polymer film surface is mated with a gloss of 20%.

One proceeds as in Example 1 but by using a composite film wherein one of the basic film surfaces is mated and has then been metallized with aluminum.

The mated surface has a 20% gloss, determined by the DIN 67530 method, by using a measurement angle of 60°.

The drawing printed on the aluminum bar (Fig. 4) does not show defects.

The definition of the printed drawing results slightly lower than that obtained in Example 2.

On the whole the obtained print results of good quality and it is therefore acceptable.

## Claims

1. A transfer printing process by colour sublimation by the bag technology, comprising the following steps:
a) covering the article surface to be printed with a composite comprising:
- a polymer film or sheet, which forms the composite basis, such as to resist without decomposing and without being deformed at the temperatures used in the colour transfer phase by sublimation, said polymer film or sheet having a thickness ranging from 6 to 100 µm and having one or both the surfaces mated, **characterized by** a gloss < 60%, determined by the DIN 67530 method with measurement angle of 85°;
- an aluminum layer, having a thickness from 0,5 to 40 nm, preferably from 1 to 20 nm having an optical density in the range 0.05-3.0, preferably 0.1-0.5, the aluminum layer being deposited on a mated surface of the polymer compound film;
- a drawing, with the respective colours, printed on the aluminum layer which is put into contact with the surface of the article to be printed;
b) longitudinal closing of the case formed by the composite and vacuum application between the composite film and the article to be printed;
c) heating at temperatures from 170°C to 240°C, preferably from 190°C to 210°C, for a time from 1 minute to 5 minutes;
d) cooling and recovery of the printed article.

2. A process according to claim 1, wherein in step b) the residual pressure ranges from 0.05 bar (5X10³ Pa) to 0.2 bar (2X10⁵ Pa), preferably it is of 0.1 bar (10⁴ Pa).

3. A process according to claims 1-2, wherein the composite is electrostatically charged.

4. A process according to claims 1-3, wherein the thickness of the polymer compound film ranges from 10 to 25 µm and the optical density of the aluminum film ranges from 0.1 to 0.5.

5. A process according to claims 1-4, wherein the gloss of the rough surface of the polymer film forming the composite basis is > 10%, measured with contact angle of 60°, and preferably it ranges from 15%, measured with angle of 60° to 55%, measured with angle of 85°, extremes included.

6. A process according to claims 1-5, wherein the polymer forming the film is selected from the following: polyesters, fluorinated resins, polyamides, polyimides, polyethers, and polyurethane resins.

7. A process according to claim 6, wherein the polymer film is formed by polyester, preferably polyethylene terephthalate, polybutylene terephthalate, glycol terephthalate.

8. A process according to claims 6-7, wherein polymer films stretched in one or both the directions, longitudinal and/or transversal, are used.

9. A process according to claims 1-8, wherein the composite film used in step a) is obtained in two steps:
- preparation of the mated polymer film;
- metallization of the mated surface of the polymer film by deposition of an aluminum layer under high vacuum conditions;
- printing of the drawing to be transferred on the side coated with aluminum.

10. A process according to claims 1-9, wherein the article to be printed has flat surfaces or it is a tridimensional article.

11. A process according to claim 10, wherein the article to be printed is formed by a compound resistant to the temperatures used in the printing process by sublimation and having surfaces which absorb the sublimable colours which are transferred from the metallized surface of the composite.

12. A process according to claim 11, wherein the surfaces of the article to be printed are coated by electrostatic painting with a layer of polymer compound preferably polyester or polyurethane thermosetting powders.

13. A process according to claims 10-12, wherein the compound of which the article to be printed is composed is selected from metals, preferably aluminum, iron, zinc, steel, cast iron, or glass, ceramic or polymer compounds.

## Patentansprüche

1. Übertragungsdruckverfahren durch Farbsublimation durch die Beuteltechnologie, umfassend die nachstehenden Schritte:
a) Bedecken der zu bedruckenden Gegenstandsoberfläche mit einem Verbundwerkstoff, umfassend:
- einen Polymerfilm oder eine Polymerfolie, der/die die Verbundwerkstoffgrundlage bildet, dergestalt, dass er/sie ohne Zersetzen und ohne verformt zu werden den bei der Farbübertragungsphase durch Sublimation verwendeten Temperaturen widersteht, wobei der Polymerfilm oder die Polymerfolie eine Dicke im Bereich von 6 bis 100 µm aufweist und eine oder beide von den Oberflächen mattiert sind, **gekennzeichnet durch** einen Glanz < 60 %, bestimmt **durch** das DIN 67530 Verfahren bei einem Messwinkel von 85°;
- eine Aluminiumschicht mit einer Dicke von 0,5 bis 40 nm, vorzugsweise 1 bis 20 nm, die eine optische Dichte im Bereich 0,05 - 3,0, vorzugsweise 0,1 - 0,5, aufweist, wobei die Aluminiumschicht auf einer mattierten Oberfläche des Polymerverbindungsfilms abgeschieden ist;
- eine Zeichnung, die mit den jeweiligen Farben auf die Aluminiumschicht gedruckt wurde, welche mit der Oberfläche des zu bedruckenden Gegenstands in Kontakt gebracht wird;
b) Längsverschließen des **durch** den Verbundwerkstoff gebildeten Fachs und Anlegen von Vakuum zwischen dem Verbundwerkstofffilm und dem zu bedruckenden Gegenstand;
c) Erhitzen auf Temperaturen von 170°C bis 240°C, vorzugsweise 190°C bis 210°C, für einen Zeitraum von 1 Minute bis 5 Minuten;
d) Kühlen und Gewinnen des bedruckten Gegenstands.

2. Verfahren nach Anspruch 1, wobei in Schritt b) der Restdruck im Bereich von 0,05 bar (5 x 10³ Pa) bis 0,2 bar (2 x 10⁵ Pa) liegt, vorzugsweise ist er 0,1 bar (10⁴ Pa).

3. Verfahren nach Ansprüchen 1 - 2, wobei der Verbundwerkstoff elektrostatisch geladen ist.

4. Verfahren nach Ansprüchen 1 - 3, wobei die Dicke des Polymerverbindungsfilms im Bereich von 10 bis 25 µm liegt und die optische Dichte des Aluminiumfilms im Bereich von 0,1 bis 0,5 liegt.

5. Verfahren nach Ansprüchen 1 - 4, wobei der Glanz der rauen Oberfläche des die Verbundwerkstoffgrundlage bildenden Polymerfilms > 10 % ist, gemessen bei einem Kontaktwinkel von 60°, und vorzugsweise liegt er im Bereich von 15 %, gemessen bei Winkel 60°, bis 55 %, gemessen bei Winkel 85°, Extrema eingeschlossen.

6. Verfahren nach Ansprüchen 1 - 5, wobei das den Film bildende Polymer aus den Nachstehenden: Polyestern, fluorierten Harzen, Polyamiden, Polyimiden, Polyethern und Polyurethanharzen, ausgewählt ist.

7. Verfahren nach Anspruch 6, wobei der Polymerfilm aus Polyester, vorzugsweise Polyethylenterephthalat, Polybutylenterephthalat, Glycolterephthalat, gebildet wird.

8. Verfahren nach Ansprüchen 6 - 7, wobei in einer oder beiden Richtungen, längs und/oder quer, verstreckte Polymerfilme verwendet werden.

9. Verfahren nach Ansprüchen 1 - 8, wobei der in Schritt a) verwendete Verbundwerkstofffilm in zwei Schritten erhalten wird:
- Herstellung des mattierten Polymerfilms;
- Metallisierung der mattierten Oberfläche des Polymerfilms durch Abscheidung einer Aluminiumschicht unter Hochvakuumbedingungen;
- Aufdrucken der auf die mit Aluminium beschichteten Seite zu überführenden Zeichnung.

10. Verfahren nach Ansprüchen 1 - 9, wobei der zu bedruckende Gegenstand ebene Oberflächen aufweist oder er ein dreidimensionaler Gegenstand ist.

11. Verfahren nach Anspruch 10, wobei der zu bedruckende Gegenstand durch eine Verbindung gebildet wird, die gegen die bei dem Druckverfahren durch Sublimation zu verwendenden Temperaturen widerstandsfähig ist und Oberflächen aufweist, die die sublimierbaren Farben absorbieren, die von der metallisierten Oberfläche des Verbundwerkstoffs überführt werden.

12. Verfahren nach Anspruch 11, wobei die Oberflächen des zu bedruckenden Gegenstands durch elektrostatisches Beschichten mit einer Polymerverbindungsschicht, vorzugsweise wärmehärtenden Polyester- oder Polyurethanpulvern, beschichtet werden.

13. Verfahren nach Ansprüchen 10 - 12, wobei die Verbindung aus der der zu bedruckende Gegenstand zusammengesetzt ist, aus Metallen, vorzugsweise Aluminium, Eisen, Zink, Stahl, Gusseisen oder Glas, keramischen oder Polymerverbindungen ausgewählt ist.

## Revendications

1. Procédé d'impression par transfert par sublimation des couleurs par la technologie de l'enveloppe («bag technology »), comprenant les étapes suivantes :
a) recouvrir la surface de l'article à imprimer avec un composite comprenant :
une feuille ou film polymère, qui forme la base du composite, de façon à résister sans se décomposer et sans se déformer aux températures utilisées dans la phase de transfert des couleurs par sublimation, ladite feuille ou ledit film polymère ayant une épaisseur comprise de 6 à 100 µm et ayant une surface ou les deux surfaces appariée(s), **caractérisé**(e) par un brillant < 60 %, déterminé par le procédé DIN 67530 avec un angle de mesure de 85° ;
une couche d'aluminium, ayant une épaisseur de 0,5 à 40 nm, de préférence de 1 à 20 nm ayant une densité optique comprise de 0,05 à 3,0, de préférence de 0,1 à 0,5, la couche d'aluminium étant déposée sur une surface appariée du film composé polymère ;
un dessin, aux couleurs respectives, imprimé sur la couche d'aluminium qui est mise en contact avec la surface de l'article à imprimer ;
b) fermer longitudinalement l'enveloppe formée par le composite et appliquer du vide entre le film composite et l'article à imprimer ;
c) chauffer à des températures de 170°C à 240°C, de préférence de 190° à 210°C, pendant une durée de 1 minute à 5 minutes ;
d) refroidir et récupérer l'article imprimé.

2. Procédé selon la revendication 1, dans lequel durant l'étape b) la pression résiduelle est de 0,05 bar (5 x 10³ Pa) à 0,2 bar (2 x 10⁵ Pa), de préférence elle est de 0,1 bar (10⁴ Pa).

3. Procédé selon les revendications 1 et 2, dans lequel le composite est chargé électrostatistiquement.

4. Procédé selon les revendications 1 à 3, dans lequel l'épaisseur du film composé polymère est comprise de 10 à 25 µm et la densité optique du film en aluminium est comprise de 0,1 à 0,5.

5. Procédé selon les revendications 1 à 4, dans lequel le brillant de la surface brute du film polymère formant la base composite est > 10 %, mesuré avec un angle de contact de 60°, et de préférence il est compris de 15 %, mesuré avec un angle de 60°, à 55 %, mesuré avec un angle de 85°, extrêmes inclus.

6. Procédé selon les revendications 1 à 5, dans lequel le polymère formant le film est sélectionné à partir des composés suivants : les polyesters, les résines fluorées, les polyamides, les polyimides, les polyéthers et les résines de polyuréthane.

7. Procédé selon la revendication 6, dans lequel le film polymère est fait en polyester, de préférence en polytéréphtalate d'éthylène, en polytéréphtalate de butylène, en téréphtalate de glycol.

8. Procédé selon les revendications 6 et 7, dans lequel des films polymères étirés dans une direction ou dans les deux directions, longitudinale et/ou transversale, sont utilisés.

9. Procédé selon les revendications 1 à 8, dans lequel le film composite utilisé à l'étape a) est obtenu en deux étapes :
- préparation du film polymère apparié ;
- métallisation de la surface appariée du film polymère en déposant une couche d'aluminium dans des conditions de vide élevé ;
- impression du dessin à transférer sur la face recouverte d'aluminium.

10. Procédé selon les revendications 1 à 9, dans lequel l'article à imprimer comporte des surfaces plates ou il s'agit d'un article à trois dimensions.

11. Procédé selon la revendication 10, dans lequel l'article à imprimer est réalisé en un composé résistant aux températures utilisées dans le procédé d'impression par sublimation et comportant des surfaces qui absorbent les couleurs sublimables qui sont transférées depuis la surface métallisée du composite.

12. Procédé selon la revendication 11, dans lequel les surfaces de l'article à imprimer sont recouvertes par peinture électrostatique avec une couche de composé polymère de préférence des poudres thermodurcissables de polyester ou de polyuréthane.

13. Procédé selon les revendication 10 à 12, dans lequel le composé dont l'article à imprimer est constitué est choisi à partir de métaux, de préférence l'aluminium, le fer, le zinc, l'acier, la fonte, ou le verre, la céramique ou les composés polymères.
